

Patented Nov. 4, 1941

2,261,295

# UNITED STATES PATENT OFFICE

2,261,295

## ARTIFICIAL TEXTILE MATERIALS

Paul Schlack, Berlin-Treptow, Germany, assignor, by mesne assignments, to Walther H. Duisberg, New York, N. Y.

No Drawing. Application September 23, 1937, Serial No. 165,333. In Germany September 30, 1936

9 Claims.

(Cl. 18—54)

My present invention relates to a process of producing fibers and films.

It is an object of the invention to provide a process by which fibers and films from organophilic polymerides may be dyed or printed in fast tints with acid wool dyestuffs, directly dyeing cotton dyestuffs, vat dyestuffs and insoluble dispersion dyestuffs. Further objects will be apparent from the detailed specification following hereafter.

It has been proposed in my copending application Ser. No. 41,500 filed September 20, 1935, to make artificial textile materials such as threads, sheets, films, bristles, horse-hair and the like from cellulose derivatives and artificial resins, soluble in organic solvents by adding to the mass synthetic resinous substances which contain reactive halogen, oxido- or sulfo-ester groups and to treat the material during or after the shaping operation or the further working up with an aminating agent or its equivalent. Films have also been produced which contain strongly degraded chloracetyl cellulose in addition to acetyl cellulose and these have been subsequently caused to react with pyridine.

The present invention consists in making valuable products of similar properties by using as additional components soluble (organophilic) sulfonic acid esters of carbohydrates, particularly cellulose and its derivatives, such as hydroxyethyl cellulose or mono-ethyl cellulose, further starch; the fibers and films obtained in the usual manner, for example by dry spinning or wet spinning, by casting on bands or the like, may be treated with aminating agents or their equivalents during the manufacture or at a later period. In this manner there are obtained products having an enhanced affinity for many dyestuff components and for agents for treating textiles, particularly those having acid groups. The increased affinity for dyestuffs is also by no means limited to acid wool dyestuffs but extends also to directly dyeing cotton dyestuffs, also to vat dyestuffs and particularly insoluble dispersion dyestuffs. These latter are particularly easily and quickly adsorbed, which is important in printing. In many cases the fastness of the dyeings, for instance towards acid gases, is considerably improved. Aminating agents, by means of which this increase of affinity may be attained, are for example: Ammonia, methylamine, dimethylamine, trimethylamine, cyclohexylamine, piperidine, morpholine, N-methylmorpholine, ethylene-diamine, tetramethyl-diamine, piperazine, N,N'-dimethylpiperazine, ethylene-imine, C-methylethylene imine, N-methylethylene imine, N-butylethylene imine, dimethylaniline, pyridine, picoline, pyridine-β-carboxylic acid methyl ester, quinoline, isoquinoline, dimethylthiazole, 4-methyl-imidazole, 60

dimethylsulfide, trimethylphosphine, ethylene thiourea, N,N'-dimethylethylene thiourea, N-cyclohexyl-N'-dimethyl thiourea, hexamethylene triamine, dimethylguanidine.

These agents, insofar as they are sufficiently volatile, may be applied in the gaseous phase, in which case the presence of moisture is frequently advantageous. Reaction can also be favored by the presence of vapors of solvents which cause swelling for example vapor of methanol, of methylene chloride, of acetone, of benzene or of alcohol. Slightly volatile or non-volatile materials may be applied in liquid form or in the form of a solution in an inert solvent, which if desired may exert a limited swelling action. Slightly volatile or non-volatile materials can also be used, when sufficiently sparingly soluble in water, in the form of emulsions or dispersions and applied or printed on the structure or to a preliminary product thereof, particularly to a web.

In order to avoid as far as possible a yellowing owing to the amination treatment it is desirable to keep the temperature of the reaction as low as is practicable and to avoid unnecessary excess of the treating agent. The presence of aldehydes or of pronounced reducing agents may sometimes be favorable in this sense.

A yellowing which may have already occurred may be removed or diminished by a bleaching agent, in particular acid bleaching agents, for instance potassium permanganate in presence of sulfuric acid, acid dispersions or arylsulfochloramides or a bleaching by exposure to light.

The reactivity of the structure may, as will appear presently, be considerably increased by the addition of further components to the film- or fiber-forming colloids before the casting or spinning which have a higher swelling capacity than that of the main material or obtain an increased degree of swelling by a moderate hydrolysis by which hydroxy groups are liberated. Such materials are, for example polymeric vinyl esters, such as vinyl formate, vinyl acetate, vinyl methoxy acetate. Especially the easily decomposed vinyl formate or a mixed polymerize having this component produces a strong increase in swelling. Hydrolysis of this kind may occur before the amination proper. Generally, however, it is preferable to conduct hydrolysis and amination in a single operation. Quite particularly active and valuable are additions of substances to the fiber-forming colloids which contain acid or latent acid groups which, for example, become freed by hydrolysis or oxidation. Hydrolytic decompositions may in this case also occur simultaneously with the amination; any oxidizing, however, must precede the amination. Suitable additional polymeric substances with acid or latent acid groups are, for

example, the polymerizates and mixed polymerizates which contain unsaturated acids, for instance acrylic acid or maleic acid, as components, especially the anhydric mixed polymerizates from maleic anhydride and vinyl derivatives, for example the mixed polymerizate from vinyl alkyl ether or vinyl carboxylic acid ester with maleic anhydride, which products are easily obtainable in the manner described in German Specification No. 540,101. Also other materials with acid groups described in my copending application Ser. No. 57,524 filed January 4, 1936 (British Patent No. 459,711), are available for the purposes of the invention.

The products which in aminated condition contain both acid and basic groups are particularly valuable from the point of view of dyeing. They may be dyed with selected members from practically all dyestuffs classes and exhibit a remarkably good stability to boiling. The affinity for dyestuffs and in many cases also to the reactivity in the amination may be further enhanced if in addition to the sulfonic acid ester of a polymeric carbohydrate a synthetic resinous substance of high molecular weight is added which at the same time contains groups capable of amination. Such substances are, for example, halogen derivatives like polyvinyl chloracetate, mixed polymerizates containing vinyl- $\alpha$ -halogen acyl radicals, polyglycide chloracetate,  $\gamma$ -chloro- $\beta$ -hydroxypropyl ethers of resinous polyhydroxy compounds, arylsulfonic acid esters or polyglycide of hydroxy-alkylated phenol formaldehyde condensation products of the "Novolak" type. Novolak is a soluble, non-hardened condensation product from phenol and formaldehyde produced by reacting the components in an acid medium. "Novolak" is a registered trade-mark.

As a basis for the textile materials having the additions prescribed by this invention there come into consideration in the first place cellulose derivatives such as cellulose esters and ethers, polyvinyl formals, mixed polymerizates from acrylic acid nitrile and vinyl alkyl ethers, or from acrylic acid amide and vinyl alkyl ethers, also polyvinyl chloride soluble in acetone.

The heterogeneous composition of fibers and films from dissimilar components results in a particularly good receptivity of the aminated fiber for dyestuffs of comparatively high molecular weight similar to that which is exhibited by products such as polyvinylchloracetate. Moreover, the embedded additional component acts as a protective against the washing out of the aminated substance in an acid treating bath. The aminated product, however, may also be fixed by after-treatment with an aldehyde or an anionic compound yielding sparingly soluble and/or hydrophobe salts.

The following examples illustrate the invention.

(1) An acetate artificial silk consisting of 90 parts of acetyl cellulose having 54.2 per cent of bound acetic acid and 10 parts of toluene sulfo-cellulose, having about 2 toluene sulfo-radicals for each glucose unit, are heated in a chamber 50 times the volume of the silk with twice the calculated proportion of pyridine for 16 hours at 80° C. In order that the evaporation of the pyridine may be uniform the liquid is absorbed in a porous body.

Instead of pyridine there may be used with like result trimethylamine, ethylene imine, N-methyl-ethylene imine, N-butyl ethylene imine. The aminated silk may be dyed with acid dyestuffs such as Alizarine Cyanine Green 5G (Schultz

Farbstofftabellen, 7th ed., vol. II, page 68), Acid Anthracene Red 5BL (Schultz Farbstofftabellen, 7th ed., vol. II, page 187), Acid Anthracene Brown RE (Schultz Farbstofftabellen, 7th ed., vol. II, page 187), in the last named case with after-chroming; the dyeings are intense and fast.

(2) A spinning solution consisting of 17.5 per cent of acetyl cellulose having 54.2 per cent of combined acetic acid, 1.5 per cent of toluene sulfo-cellulose having 2 toluene sulfo-radicals for each glucose unit, 1 per cent of the mixed polymerizate from 1 mol vinyl methyl ether and 1 mol maleic anhydride and 80 per cent of acetone is spun by the dry spinning process. The silk obtained after amination with N-butylethylene imine is dyed intensely by acid dyestuffs at 70-80° C.

(3) A spinning solution consisting of 18 per cent of acetyl cellulose, 5 per cent of polyvinyl chloracetate and 5 per cent of toluene sulfo-cellulose with 2 acyl radicals for each glucose unit is spun by the dry spinning process. The silk has approximately the normal physical properties of an acetate silk from the same acetate without the addition of a substance capable of being aminated. By treatment with pyridine vapor in the manner described in Example 1 there is obtained a textile material which can be dyed fast intense tints with dyestuffs having acid groups or with dyestuff derivatives such as Indigosol Green (Schultz Farbstofftabellen, 7th ed., vol. II, page 133) by the nitrite method.

(4) A mixture of 80 parts of ethyl cellulose having 41 per cent of ethoxyl and 20 parts of toluene sulfo-cellulose having about 2 toluene sulfo-groups for each glucose unit is dissolved in a mixture of methylene chloride and alcohol (85:15) and cast to form films. After amination with pyridine or dimethyl thiazole the films may be dyed intensely by means of acid dyestuffs.

(5) There is spun by the dry spinning process a solution of 17.5 parts of acetyl cellulose having 54.2 per cent of combined acetic acid, 1.5 per cent of toluene sulfo-cellulose having 2 acyl radicals for each glucose unit and 1 per cent of the mixed polymerizate from 1 mol vinyl chloride and 1 mol maleic anhydride hydrolyzed to yield the polymeric acid, in 80 parts of acetone (strictly speaking 79.15 if the water introduced together with the mixed polymer is calculated). By treatment with vapor of pyridine the silk acquires basic properties. The mixed polymerizate is worked into the spinning solution in the form of an aqueous solution of 60 per cent strength.

(6) A solution of 17.5 parts of acetyl cellulose, 5 parts of polyvinyl acetate and 5 parts of ethane-sulfo-cellulose in a mixture of methylene chloride and methanol (85:15) is spun as artificial silk. By treatment from 12 hours with twice the calculated proportion of N-methylmorpholine in toluene at 60° C. the silk is aminated and may now be dyed with acid wool dyestuffs and with many substantive dyestuffs.

(7) A solution containing 17.4 per cent of acetyl cellulose having 54.2 per cent of combined acetic acid, 0.8 per cent of toluene sulfo-cellulose, 0.8 per cent of polyvinyl chloracetate and 0.8 per cent of the mixed polymerizate from 1 mol vinyl methyl ether and 1 mol maleic anhydride is spun. The silk thus obtained may be dyed in presence of 7 per cent of cyclohexyl dimethyl thiourea at 70-80° C. with 3 per cent of Alizarine Cyanine Green G Extra (Schultz Farbstofftabellen, 7th ed., vol. I, page 532); strong tints are produced.

(8) A solution of acetyl cellulose containing 7.5 per cent of toluene sulfo-cellulose and 2.5 per cent of the mixed polymerizate from vinyl formate and maleic anhydride is spun and the fiber is treated directly after it has left the spinning cell with a solution of 15 per cent strength of isoquinoline in dilute acetone. After evaporation of the acetone the fiber is heated at 70° C. in a closed chamber for some time; it is then cut to staple and further worked up in the usual manner.

(9) A spinning solution containing 18 per cent of acetyl cellulose having 54.2 per cent of combined acetic acid and 4 per cent of an acetyl-toluene-sulfonyl-cellulose containing about 2 acetyl radicals and about 0.7 toluene sulfonyl radicals for each glucose unit, the solvent being a mixture of methylene chloride and ethanol (85:15), is spun by the dry spinning process to form artificial silk. The silk is then aminated by means of trimethylamine; it may then be dyed deep tints with acid dyestuffs, for instance Orange II (Schultz Farbstofftabellen, 7th ed., vol. I, page 86), or Alizarine Direct Blue A (Schultz Farbstofftabellen, 7th ed., vol. II, page 9).

(10) A solution of hydroxyethyl cellulose acetate in acetone which contains 10 per cent of toluene sulfo-starch is worked up into a film from a mixture of methylene chloride and alcohol (80:20). The film is aminated by treatment with a solution of pyridine in toluene, whereupon it exhibits good affinity for acid dyestuffs.

(11) 18 parts of acetyl cellulose having 52.5 per cent of combined acetic acid and 2 parts of the ether ester from dimethyl cellulose and diethylaminosulfochloride, in a mixture of methylene chloride and alcohol (80:20) is cast into the form of a film. The ether ester is obtained by heating the ether with the acid chloride in an indifferent solvent in presence of an agent which binds hydrogen halide.

(12) A 16 per cent solution of 92 parts cellulose acetate having 59.2 per cent of bound acetic acid and 8 parts phenylsulfonyl starch in acetic acid is spun by the wet spinning process. The silk obtained is treated with a 4 per cent solution of benzylamine in aqueous pyridine of 25 per cent strength at 75° C. for one hour. The silk is aminated and slightly saponified and can now be dyed with many acid dyestuffs. By addition of swelling agents to the dye bath the number of dyestuffs available is increased.

What I claim is:

1. A process which comprises preparing a solution of cellulose acetate, adding thereto 10 parts of the weight of the cellulose acetate of toluene-sulfo cellulose, spinning artificial silk therefrom by the dry spinning process, heating the resulting silk at about 80° C. for about half a day to a day in an atmosphere containing pyridine vapor.

2. A process which comprises preparing a solution in acetone comprising mainly acetyl cellulose, a comparatively small amount of toluene-sulfo cellulose having in its molecule 2 toluene sulfo-radicals per glucose unit and a comparatively small amount of a mixed polymerizate from vinyl methyl-ether and maleic anhydride, spinning fibers from said solution by the dry spinning process, and treating said fibers with an alkylene imine.

3. A process which comprises preparing a solution of about 18 per cent of acetyl cellulose, 5 per cent of polymerized vinyl chloracetate and 5 per cent of toluene-sulfo cellulose, spinning fibers from said solution, and treating said fibers at 80° C. for a considerable time with dimethylthiazole.

4. A process which comprises preparing a solution of a polymeric organophilic colloid selected from the group consisting of cellulose derivatives and fiber-forming synthetic resins, adding to the said solution a soluble ester of a polymeric carbohydrate with a sulfonic acid, forming fibers or foils from said solution, and reacting said fibers and foils with a compound selected from the group consisting of amines and amine derivatives.

5. A process which comprises preparing a solution of a polymeric organophilic colloid selected from the group consisting of cellulose derivatives and fiber-forming synthetic resins, adding to the said solution a soluble ester of a polymeric carbohydrate with a sulfonic acid, forming fibers or foils from said solution, and reacting said fibers and foils with a compound selected from the group consisting of amines and amine derivatives in gaseous condition.

6. A process which comprises preparing a solution of a polymeric organophilic colloid selected from the group consisting of cellulose derivatives and fiber-forming synthetic resins, adding to the said solution a soluble ester of a polymeric carbohydrate with a sulfonic acid, adding further to the said solution a synthetic resinous substance containing in its molecule an alkylating group, forming fibers and films from said solution, and treating said fibers and films with a compound selected from the group consisting of amines and amine derivatives.

7. A process which comprises preparing a solution of a film-forming polymeric organophilic colloid selected from the group consisting of cellulose derivatives and fiber-forming synthetic resins, adding to the said solution a soluble ester of a polymeric carbohydrate with a sulfonic acid, adding further to the said solution a polymeric substance having a higher swelling capacity in water than said first named film-forming compound, forming fibers or films from said solution, and treating said fibers or films with a compound selected from the group consisting of amines and amine derivatives.

8. A process which comprises preparing a solution of an organic cellulose derivative, adding to said solution a soluble ester of a polymeric carbohydrate with an organic sulfonic acid, forming fibers or foils from said solution, and treating said fibers or foils with a compound selected from the group consisting of amines and amine derivatives.

9. Artificial fibers and films made of an organophilic colloid which has incorporated and fixed within the body of the fibers and films a substance consisting of the reaction product of a soluble ester of a polymeric carbohydrate selected from the class consisting of cellulose and starch with a sulfonic acid, and a compound selected from the group consisting of amines and amine derivatives.

PAUL SCHLACK.